

July 9, 1946.

C. G. VAN BRUNT  
ELECTRICAL CONTACT BRUSH

2,403,471

Filed June 21, 1941



Inventor:  
Charles G. Van Brunt,  
by Harry E. Dunham  
His Attorney.

Patented July 9, 1946

2,403,471

# UNITED STATES PATENT OFFICE

2,403,471

## ELECTRICAL CONTACT BRUSH

Charles G. Van Brunt, Schenectady, N. Y., assignor to General Electric Company, a corporation of New York

Application June 21, 1941, Serial No. 399,125

14 Claims. (Cl. 171—325)

1

My invention relates to electrical contact elements and particularly to improved contact brushes and methods of making the same.

An object of my invention is to provide an improved electrical contact element.

Another object of my invention is to provide an improved electrical contact element formed of a porous block of electrically conductive material provided with a lubricant for the contact surface thereof.

A further object of my invention is to provide an improved method of making an electrical contact element.

Further objects and advantages of my invention will become apparent and my invention will be better understood from the following description referring to the accompanying drawing, and the features of novelty which characterize my invention will be pointed out with particularity in the claims annexed to and forming part of this specification.

The single figure in the drawing illustrates a contact brush for a dynamo-electric machine embodying my invention and made in accordance with my improved method of manufacture.

It has been found that under normal atmospheric conditions with average humidity, atmospheric water vapor provides the best lubricant for the contact surface of carbon and metal-graphite brushes. It has also been found that electrical contact elements made of porous blocks of finely divided electrically conductive material, such as carbon or metal and graphite brushes, tend to wear away very rapidly in dry atmospheres. In the past, different lubricants have been suggested for minimizing the friction of the contact surface of the brushes and thereby improving the life of the contact element. Most of the lubricants which have been suggested disadvantageously change the electrical characteristics of the brush or combine with the contact element, through vibration or otherwise, to form substances which impede the free movement of the contact element on its guide member or brush holder, thereby decreasing the efficiency of operation of the combination. It has been found, however, that by impregnating a porous block of electrically conductive material with a humectant, such as a polyhydric alcohol or an alcohol-ether, or mixtures of these, in at least a portion of the block, lubrication is provided for the contact surface thereof which greatly increases the life of the porous block. Furthermore, I have found that under certain conditions and for certain types of materials, the contact element is

2

improved by applying to the sides thereof a coat of relatively thin material which will not itself form interfering substances with the material with which it comes into contact, and which also prevents penetration or exudation of the impregnant through the coating to form such interfering substances when the brush vibrates and moves on its guiding surface, as has been herein described.

10 In the drawing, I have shown an electrical contact element including a porous block 10 of bonded finely divided electrically conductive material, such as carbon, graphite, metal-graphite, or other similar material conventionally used in the manufacture of contact elements, such as commutator and slip-ring brushes. A terminal clip 11 is secured to the porous block 10 by a rivet 12 and an electrically conductive pigtail member 13 is secured to the terminal clip 11 and to a connecting terminal element 14 for conducting current between a brush holder connector and the contact element block 10. In order to provide a lubricant to the contact surface 15 of the porous block 10, a portion of the block below the terminal clip 11, or the entire porous block 10, is impregnated with a hygroscopic material, such as a polyhydric alcohol solution. Among the polyhydric alcohols which have been found to provide an efficient lubricant for the contact surface of the brush 10, the ethylene glycols have been found to be particularly efficient. Mixtures of different polyhydric alcohols also have good lubricating properties. These impregnants are highly hygroscopic and water soluble and have a relatively wide liquid state temperature range. Generally, they also have the desirable properties of a relatively high flash point and a relatively low vapor pressure at normal contact element operating temperatures. For certain types of electrically conductive materials, such as carbon, electrographitic, or natural graphite brushes, a solution of from 10% to 30% of nonaethylene glycol,



45 in water has been found to be a very efficient impregnant, especially if the metal content of the brush is 50% or less. For contact elements wherein the porous material comprises a very large amount of metal, 60% or more, an impregnant comprising 40% to 60% nonaethylene glycol and 20% to 30% polyolefin glycol in water is a very efficient lubricant.

50 In forming my improved contact elements, it has been found desirable to degas the porous

block by subjecting it to a relatively low pressure and then impregnating the degassed block with the lubricant, after which excess impregnant is removed from the block, and, in certain cases, a relatively thin coating of material, which does not react with the impregnant and is otherwise stable under operating conditions, is applied to the sides of the dried block. In degassing the porous block, the contact element is immersed in a solution of the impregnant, such as a 20% to 40% solution of nonaethylene glycol in water or benzene, and the block is subjected to a relatively low pressure in this solution for one to two hours, such that the water or benzene boils, removing the gas from the porous block. After this treatment, a part or the whole of the porous block is impregnated at substantially atmospheric pressure with a solution of polyhydric alcohol in water or benzene for from one to two hours. Excess impregnant then is removed from the outside of the block in any suitable manner, as by wiping or draining. The block may then be dried at a temperature between 70° and 120° C. to remove excess water from the brush. As stated above, with certain porous materials, it is desirable to provide a very thin coating of non-paste forming material over the sides of the block. I have found that a thin coating of certain lacquers applied to the sides of the block provides an efficient surface which will not react with the impregnant or other adjacent materials, even after long periods of use and vibration over a supporting or guiding surface and will effectively prevent the penetration or exudation of impregnant through the coating. This lacquer preferably is of an air-drying type, such as acetone-soluble cellulose nitrate or cellulose acetate, which provides a relatively low-friction guiding surface for the brush on its brush holder and effectively prevents sticking of the brush in the holder. I have found that a lacquer having a viscosity of three or four times that of water provides a very satisfactory coating. Acetone-soluble cellulose acetate dissolved in the solvent in proportions of about five grams of solid cellulose acetate to 95 cc. of acetone gives a lacquer of the above type. The desired impenetrable surface coating is formed on the sides of the block 10 by dipping or immersing the block for fifteen seconds to a minute in the lacquer, then draining and wiping or shaking off excess lacquer. This fills the pores on the sides of the brush and prevents exudation of the impregnant. Cellulose nitrate lacquer applied in this same manner also has given very good results. Other lacquers also have proved successful when applied to the block in relatively thin coatings. The chief requisite of the lacquer coating is that it must not react with the impregnant and must prevent exudation of the impregnant from the surface of the brush.

While I have illustrated and described particular embodiments of my invention, modifications thereof will occur to those skilled in the art. I desire to be understood, therefore, that my invention is not to be limited to the particular arrangements disclosed, and I intend in the appended claims to cover all modifications which do not depart from the spirit and scope of my invention.

What I claim as new and desire to secure by Letters Patent of the United States is:

1. An electrical contact element including a porous block of finely divided electrically conductive material, at least a portion of said block being impregnated with a polyhydric alcohol solu-

tion providing a lubricant for the contact surface of said element, and a coating on the sides of said block, said coating being impenetrable by said impregnant.

2. An electrical contact element including a porous block of finely divided material, at least a portion of said block being impregnated with an alcohol-ether solution providing a lubricant for the contact surface of said element, and a thin coating on the sides of said block, said coating being impenetrable by said impregnant.

3. An electrical contact element including a porous block of finely divided electrically conductive material, at least a portion of said block being impregnated with a polyhydric alcohol solution providing a lubricant for the contact surface of said element, and a lacquer coating on the sides of said block.

4. An electrical contact element including a porous block of finely divided material at least a portion of said block being impregnated with a polyhydric alcohol solution providing a lubricant for the contact surface of said element, and an air drying lacquer coating on the sides of said block.

5. An electrical contact element including a porous block of finely divided material, at least a portion of said block being impregnated with a polyhydric alcohol solution providing a lubricant for the contact surface of said element, and a cellulose acetate lacquer coating on the sides of said block.

6. An electrical contact element including a porous block of finely divided material, at least a portion of said block being impregnated with a polyhydric alcohol solution providing a lubricant for the contact surface of said element, and a cellulose nitrate lacquer coating on the sides of said block.

7. The method of making an electrical contact element including forming a porous block, degassing the porous block, impregnating at least a part of the degassed porous block with a polyhydric alcohol solution, and applying to the sides of the impregnated block a relatively thin coating of material impenetrable by the impregnant.

8. The method of making an electrical contact element including forming a porous block of electrically conductive material, degassing the porous block by subjecting it to a relatively low pressure, impregnating at least a part of the degassed porous block with nonaethylene glycol, removing excess impregnant from the block, and applying to the sides of the block a relatively thin coating of material impenetrable by the impregnant.

9. The method of making an electrical contact element including forming a porous block of electrically conductive material, degassing the porous block by subjecting it to a relatively low pressure, impregnating at least a part of the degassed porous block with a polyhydric alcohol solution, removing excess impregnant from the block by draining and by drying, and applying a relatively thin coating of lacquer to the sides of the dried block.

10. The method of making an electrical contact element including forming a porous block of electrically conductive material, degassing the porous block by subjecting it to a relatively low pressure, impregnating at least a part of the degassed porous block with a solution of nonaethylene glycol and polyolefin glycol, removing excess impregnant from the block, applying a rel-

atively thin coating of lacquer to the sides of the dried block, and removing excess lacquer.

11. The method of making an electrical contact element including forming a porous block of electrically conductive material, degassing the porous block by subjecting it to a relatively low pressure, impregnating at least a part of the degassed porous block with a polyhydric alcohol solution, removing excess impregnant from the block by draining and by drying at a temperature substantially between 70° and 120° C., applying a relatively thin coating of lacquer to the sides of the dried block, and removing excess lacquer by wiping and by drying at a temperature of substantially between 75° and 120° C. for substantially an hour.

12. The method of making an electrical contact element including forming a porous block of electrically conductive material, degassing the porous block by subjecting it to a relatively low pressure for from one to two hours, impregnating at least a part of the degassed porous block with a solution of nonaethylene glycol in benzene for from one to two hours, removing excess impregnant from the block by draining and by drying at a temperature between 70° and 120° C., applying a relatively thin coating of lacquer to the sides of the dried block, and removing excess lacquer by wiping and by drying at a temperature of between 75° and 120° for substantially an hour.

13. The method of making an electrical contact element including forming a porous block of electrically conductive material, degassing the po-

rous block by subjecting it to a relatively low pressure for from one to two hours, impregnating at least a part of the degassed porous block with a solution of nonaethylene glycol in water for from one to two hours, removing excess impregnant from the block by draining and by drying at a temperature between 70° and 120° C., applying a relatively thin coating of lacquer to the sides of the dried block, and removing excess lacquer by wiping and by drying at a temperature of between 75° and 120° C. for substantially an hour.

14. The method of making an electrical contact element including forming a porous block of finely divided metallic and graphitic electrically conductive material, degassing the porous block by immersing in a 20% to 40% solution of nonaethylene glycol in water and subjecting the block for one to two hours to a relatively low pressure such that the water of the solution boils, impregnating at least a part of the degassed porous block at substantially atmospheric pressure with a 10% to 30% solution of nonaethylene glycol in water for from one to two hours, removing excess impregnant from the block by draining and by drying at a temperature between 70° and 120° C., applying a relatively thin coating of lacquer to the sides of the dried block, and removing excess lacquer by wiping and by drying at a temperature of between 75° and 120° C. for substantially an hour.

CHARLES G. VAN BRUNT.